

## UNITED STATES PATENT OFFICE

2,086,178

## WATERMARKING PELLICLE

James E. Snyder, Kenmore, N. Y., assignor, by  
mesne assignments, to E. I. du Pont de Ne-  
mours & Company, Wilmington, Del., a corpo-  
ration of Delaware

No Drawing. Application January 15, 1934,  
Serial No. 706,710

5 Claims. (Cl. 18—48)

This invention relates to a new article of manufacture. The invention relates to a process of manufacturing the new article. More particularly the invention relates to a process of manufacturing a watermarked pellicle of non-fibrous cellulosic character. Still more particularly the invention relates to the manufacture of watermarked regenerated cellulose pellicles.

The watermarking of paper is an old and well-known process by which a sheet of paper carries a mark, design, or picture substantially invisible by reflected light but visible by transmitted light. The watermarking process has enabled paper manufacturers to identify their products and to prevent the deception of the public.

There is on the market a non-fibrous, non-porous, transparent tissue, ordinarily used for wrapping purposes, comprising regenerated cellulose film. Other sheets of similar non-fibrous character have been made from cellulose esters such as cellulose acetate, and from cellulose ethers. No satisfactory method has been developed for imparting to these sheets a mark similar in character to a watermark such as is used in paper. Attempts have been made to impress a mark upon the finished sheet by moistening and die-pressing but the results have been unsatisfactory for various reasons, for example, the mark lacks suitable permanence. Attempts to mark the sheeting in manufacture after it has been at least partially coagulated but before it has been completely regenerated have not been entirely successful because the pellicle shrinks greatly during drying and the impression is distorted and in some cases disappears.

One object of this invention pertains to the production of a dense, smooth, non-porous, non-fibrous, preferably transparent cellulose film having imparted thereto permanent indicia, such as numbers, letters and the like. Another object of the invention pertains to the production of films of this character, comprising regenerated cellulose. A further object of the invention comprises production of film of the character described carrying indicia similar in appearance and character to the "watermarking" used in paper. Other objects of the invention will appear herein-after.

The invention will be described most particularly in its application to the manufacture of regenerated cellulose pellicles. It is to be understood that this description is illustrative and not limitative.

In the manufacture of regenerated cellulose sheeting by one method, a viscous solution is

forced through a thin, elongated orifice of uniform width into and beneath the surface of a coagulating bath wherein the viscous is precipitated and the regeneration commenced and sometimes completed. The pellicle thus formed is passed through additional regenerating, washing, desulfuring, and glycerinating baths, and occasionally through other baths designed to accomplish particular ends, and from these baths is passed to the driers. In the ordinary pellicle manufacturing machine the drier consists of a series of heated rollers over the surfaces of which the pellicle travels, being wound up at the end in a dried and completely usable condition.

It is my discovery that if the pellicle be impressed when it is partially dried, for instance, by impression with a die having raised figures or designs, it will retain the impression permanently. It is desirable that the impression be made at a particular stage in the drying. The impression, for all practical purposes, must be made upon the pellicle when the moisture content of the pellicle has been reduced to between about 45% and about 190% of the weight of the dry pellicle plus glycerine (or other softener). Preferably, the impression should be made at a moisture content of about 100% because better and more uniform results are obtained. However, it is possible to obtain advantages of the invention occasionally at moisture percentages of 45% and even lower and moisture percentages of 190% or even higher. When the impressions are made with moderate pressure at a moisture content less than about 45%, the impressions are so faint as to be either invisible or scarcely discernible. Impressions made at moisture contents above about 190% become distorted during drying and unless the pressures used are very high gradually fade out, being substantially unrecognizable or entirely invisible at the completion of the manufacturing operation.

It should be understood that it is not desirable to use heavy pressures to impress the pellicle because heavy pressures tend to puncture or to rupture the pellicle. In ordinary practice, a die roller, bearing on its surface a raised insignia or design, will be placed in contact with a dryer roller. The pellicle will be passed between the impressing roller and the dryer roller and will receive the impression from the die. It is necessary that the pressure exerted by the die against the pellicle be sufficient to impart to the pellicle a permanent mark. The actual pressure used for impressing a pellicle can readily be determined by experiment. The magnitude

5

10

15

20

25

30

35

40

45

50

55

of the pressure will depend somewhat on the size and design of the dies, the number of impressions imparted to the pellicle in a unit of area, and upon the material of which the die is made. 5  
5 Similarly, the pressure used will vary, depending upon the type of pellicle which is being manufactured. The watermark can be given an embossed appearance by impressing the sheet with a die against a roughened surface. For example, a satisfactorily embossed appearance can be obtained by covering the dryer roll, with which the roller carrying the die contacts, with a fine mesh screen. The embossed watermark can be seen by reflected as well as by transmitted 10 light. An embossed surface can also be obtained by impressing against a smooth roller with a die having an embossed or roughened surface. If both the die and the supporting surface are smooth, the watermark is visible by reflected 15 light at certain angles only.

This invention may be applied to the marking of tubes, caps, bands, and other pellicles of regenerated cellulose in the same manner as has been described for sheets of regenerated 20 cellulose.

The invention is applicable to the manufacture of cellulose ester and cellulose ether pellicles obtained from aqueous solution. In the manufacture of cellulose acetate, for example, cellulose acetate dissolved in a suitable aqueous 30 solution may be cast into an aqueous coagulating bath. The film is then passed through suitable washing tanks and led to the dryer. The impressing roller is arranged to bear against the pellicle in a position where enough of the water will have been removed from the pellicle to insure the pellicle retaining the mark after complete drying.

The die used to impress the pellicle is preferably made of elastic vulcanized rubber, since this material is durable, conforms by reason of its resilience to the contacted surface, and has less tendency to injure the sheet than other materials. Other materials than rubber can be used however, for example, wood, metal and artificial resins. These latter materials, however, since they are non-resilient, have a tendency to puncture or rupture the pellicle. When the impression is applied manually, the tendency of dies made of non-resilient material to rupture the pellicle can be regulated to a great degree by a careful operation. However, when the impressing is done by machine, for example, by means of a die roller, means should be used to overcome the rupturing tendency of non-resilient dies. Such means comprises suitably mounting the roller so as to permit it to ride freely on the pellicle, the pressure in this instance being imparted by the weight of the roller, or by using spring mountings, counterweights, or similar mechanisms to accomplish the same results.

It is evident from the above description that my invention comprises a highly satisfactory

method for permanently watermarking transparent, non-fibrous, non-porous, cellulosic pellicles. The term "watermark", as it has been used in describing this invention, is intended to signify a transparent mark resembling the watermark imparted to paper, which is permanently imparted to the cellulosic pellicle, is visible by transmitted light and which results from a treatment of the pellicle during manufacture. 5

An advantage of this invention resides in its 10 simplicity, great efficiency and inexpensiveness. A further advantage of the invention resides in the fact that the watermarks imparted to the cellulosic pellicles are clear, visible, undistorted, permanent and leave the sheets or pellicles of 15 unimpaired strength and quality.

This invention is of primary importance in treating regenerated cellulose pellicles which are preferably, though not necessarily, transparent. The invention may also be applied to the watermarking of similar films obtained from other cellulosic materials by wet methods, e. g., cellulose ester and cellulose ether pellicles obtained from aqueous solution. 20

As many apparently widely different embodiments of this invention may be made without departing from the spirit and scope thereof, it is to be understood that I do not limit myself to the specific embodiments thereof except as defined in the appended claims. 25

I claim:

1. An article of manufacture comprising a pellicle of regenerated cellulose bearing a watermark, said watermark having been imparted to the sheet by impressing the pellicle during the 30 drying thereof and while the pellicle still retained from 45 to 190% moisture based on the weight of the dry pellicle plus softener.

2. The method of manufacturing a marked pellicle of regenerated cellulose, which comprises casting, coagulating and regenerating the pellicle, partially drying the same, impressing the pellicle with a die while the pellicle has a moisture content of between 45% and 190%, based on the weight of the dry pellicle plus softener, 40 and completing the drying.

3. In the method of manufacturing watermarked pellicles of regenerated cellulose which comprises casting, coagulating, regenerating, softening and drying a pellicle, the step which comprises die-pressing the pellicle while its moisture content is 45% to 190% based on the weight of the dry pellicle plus softener. 50

4. A method of imparting a watermark on a non-fibrous, transparent cellulosic pellicle comprising die-pressing the pellicle while its moisture content is 45-190%, based on the weight of the dry pellicle, plus the softener. 55

5. A method of imparting a watermark on a regenerated cellulose pellicle comprising die-pressing the pellicle while its moisture content is 45-190%, based on the weight of the dry pellicle, plus the softener. 60

JAMES E. SNYDER.